

## UNITED STATES PATENT OFFICE

2,001,951

PHOTOGRAPHIC PRINTING EMULSION  
AND ITS PRODUCTION

William Ambler Berry, Knutsford, England, assignor to Ilford Limited, Ilford, England, a British company

No Drawing. Application March 15, 1934, Serial No. 715,779. In Great Britain March 22, 1933

8 Claims. (Cl. 95—6)

This invention comprises improvements in or relating to photographic emulsions of the development type.

Photographic emulsions may be divided into two main types. One type comprises the printing-out emulsions which consist essentially of silver chloride together with an excess of a soluble silver salt such as silver nitrate or a silver salt of an organic acid, e. g. silver citrate, lactate, or oxalate. With such emulsions an image is obtained simply by exposure to light. The other type comprises the development emulsions which consist chiefly of silver chloride, silver bromide or combinations thereof, and do not contain any soluble silver salts. A development emulsion does not, even on prolonged exposure to light, give a useful visible image, but requires development after exposure (insufficient in itself to give a visible image) to produce the useful visible image.

With certain development emulsions including those of the so-called "gaslight" type one usually obtains an image which is substantially black and it is known to incorporate substances in these emulsions or to vary the conditions of development in order to modify the quality of the blackness of this image produced by development. Also, the tone or colour of such developed images may be modified by treatment in a toning bath to give an image of substantially different chemical composition from that of the developed image, for example in a sulphide solution which gives sepia tones by conversion of the silver image into silver sulphide.

It is an object of the present invention to provide a development emulsion which has self-toning properties and produces upon development and fixation a toned image comparable with one obtained on printing out paper when printed and toned in the usual way. British Patent No. 10,051 of 1906 describes a self-toning silver chloride printing-out paper prepared from an emulsion containing chloride of gold to which a salt or salts of lead have been added for the purpose of improving the toning properties. That specification, however, is concerned only with printing-out emulsions, while the present invention, on the other hand, is concerned only with development emulsions which are distinguished from printing-out as indicated above.

The present invention comprises a self-toning development emulsion in which the light-sensitive salt consists mainly or exclusively of silver chloride without any soluble silver salts and which contains self-toning ingredients comprising a

gold salt and a lead salt with or without a thiocyanate.

In putting the present invention into effect it is preferable when the thiocyanate is omitted from the emulsion that it should be added to the fixing bath.

The invention also includes a process for the production of a photographic development emulsion comprising forming an emulsion containing essentially gelatine and silver chloride precipitated in situ and then adding a toning agent.

The invention further includes a method of producing a toned image which consists in exposing to light a paper bearing a self-toning development emulsion, developing the exposed paper and finally toning and fixing the image in one operation by immersing the print in a solution of sodium thiosulphate.

In U. S. specification Ser. No. 631,272 photographic emulsion is described having printing-out self-toning properties, that is to say, which on exposure to light produces a visible image which on subsequent treatment in a fixing bath gives an image toned according to duration of the treatment. According to the specification an essential ingredient of the emulsion is a salt of manganese. Further, the specification states that the emulsion is also amendable to the production of a self-toned image by development and fixing.

It has now been found that the omission of the manganese salt in the preparation of such an emulsion, whilst destroying the printing out properties of the emulsion, does not impair the self-toning properties and that images produced by the action of light on these emulsions can be developed and subsequently toned in a fixing bath.

The theories underlying the nature of the phenomena imparting self-toning qualities to developed photographic images are not at present thoroughly understood and therefore limiting conditions for producing emulsions yielding suitable developed images cannot be given. It has, however, been found during the course of experiments that emulsions in accordance with the present invention containing silver chloride in the form of very fine grains give particularly good results, since this on development in certain well-known developers give what are known as warm-toned images, that is, images which are of a red or yellowish-red colour.

On the other hand, it has been found that other development emulsions containing substances for modifying the quality of the black-

ness of the image during development are not suitable, as the added substance appears to interfere with the toning properties of the toning ingredients when these are added to the emulsion 5 in accordance with the present invention.

A preferred process for the manufacture of a self-toning development emulsion according to the present invention comprises forming an emulsion consisting essentially of silver chloride 10 and gelatine by precipitating the silver chloride in situ by adding a precipitating chloride (for example a chloride of sodium, ammonium, strontium, lithium or manganese) to a solution of a soluble silver salt such as silver nitrate, 15 then washing the emulsion to remove the residual nitrate (i. e. of sodium, ammonium or the like) and finally incorporating self-toning ingredients in the washed emulsion.

The following is a specific description, by way 20 of example only, of one method of manufacturing an emulsion according to the invention:

A solution comprising gelatine, water, citric acid and silver nitrate was made up at 110° F. and to this was added a quantity of a solution of 25 manganese chloride more than sufficient to precipitate all the silver in the form of silver chloride. The quantities were as follows:

|                        |      |      |
|------------------------|------|------|
| Gelatine               | 24   | gms. |
| Water                  | 200  | cc.  |
| 2½N citric acid        | 5    | cc.  |
| 2½N silver nitrate     | 10.0 | cc.  |
| 2½N manganese chloride | 11.0 | cc.  |

Emulsification was effected in the usual way and 35 the emulsion shredded. The emulsion was then washed for one hour in 6 changes of water and melted out at 110° F.

A gold solution was made up by adding ammonium thiocyanate to sodium gold chloride in 40 the presence of gum arabic, the following proportions being employed:

|                                                 |      |      |
|-------------------------------------------------|------|------|
| 6% gum arabic solution                          | 7.5  | ccs. |
| 25% sodium gold chloride (NaAuCl <sub>4</sub> ) | 0.75 | ccs. |
| 1.6% ammonium thiocyanate                       | 7.5  | ccs. |

45 and this solution was then added to the above washed emulsion, to which the following substances were also added:

|                    |      |      |
|--------------------|------|------|
| 50 2½N citric acid | 5    | ccs. |
| Gelatin            | 6    | gms. |
| Methylated spirit  | 20   | ccs. |
| 5% chrome alum     | 2.5  | ccs. |
| 25% lead nitrate   | 2.0  | ccs. |
| 40% formalin       | 0.75 | ccs. |

The volume was made up to 350 ccs. This formula gives a slow emulsion which may be increased in speed by the addition of suitable amounts of the agents normally used for increasing speed, e. g. thiosinamine or sensitizing dyes. 60

During the emulsification step described above silver chloride is precipitated from the solution of silver nitrate by the manganese chloride, and the soluble manganese nitrate formed is removed 65 by the washing which also removes any excess manganese chloride remaining. It will be noted that the emulsion is washed before the gold compound and other finals are added to it. It will be appreciated that the substances added at the 70 same time as the self-toning ingredients are those normally added to photographic emulsions to impart hardness to the gelatine and such desirable properties.

The emulsion is coated on paper in the usual 75 manner.

Conveniently the following procedure is adopted in preparing the print. After an exposure to artificial light, comparable in duration to that given to ordinary gaslight papers, for example, for 4 or 5 seconds to a 100 watt ½-watt type lamp at a distance of six inches with a normal negative, the paper is passed direct, i. e. without preliminary washing, into a developer of the formula:—

|                             |      |      |
|-----------------------------|------|------|
| Adurol                      | 1.25 | gms. |
| Sodium sulphite (crystals)  | 5    | gms. |
| Sodium carbonate (crystals) | 10   | gms. |
| Potassium bromide           | 0.5  | gms. |
| Water                       | 550  | ccs. |

10  
15

During development a reddish image is produced. Thereafter the print is immersed in an acid stop bath (e. g. a one per cent solution of hydrochloric acid) for one minute, then washed for two minutes, and finally transferred to the fixing bath in 20 which toning takes place. This bath may conveniently comprise a 30% solution of sodium thiosulphate to which may, if desired, be added a small proportion of ammonium thiocyanate. Immersion in the toning and fixing bath is continued until the desired shade of colour has been reached, and the print is then withdrawn and washed thoroughly before drying. The actual tone obtained depends upon the duration of treatment in the fixing bath and with normal 30 negatives immersion of about five minutes will produce a medium tone, whilst the coldest tones are obtained after immersion for a period of about twelve minutes. Slower toning and slightly warmer tones can be obtained by using a 35 weaker fixing bath of approximately 20% strength. The actual tone may be modified by the addition of more or less thiocyanate to the fixing bath.

Still colder tones may be obtained if desired 40 by treating the print after removal from the developing bath and before fixing, in a solution of common salt with or without potash alum until the colour has reached the desired tone, the print then being removed and fixed in thiosulphate in the ordinary way, or alternatively common salt may be added to the fixing bath. 45

If in the manufacture of the emulsion according to the formula given herein, the manganese chloride is replaced by sodium, ammonium, lithium or strontium chloride, an emulsion of substantially the same properties will be obtained. Where sodium, ammonium and lithium chlorides, or chlorides of other metals which do not produce a scum of insoluble carbonate 50 in the developer, are employed, the complete process may be carried out with some measure of success even if the emulsion is not washed before the addition of the gold and other finals, and there is no preliminary washing of the print 55 before development. However, although the toning process is not prevented by the presence of the nitrates of sodium, ammonium and lithium or the like, improved results are obtainable when these are removed. 60

Variation in the tone and in the rate of toning may be obtained by varying the amount and/or composition of the toning agents added to the emulsion.

I claim:

1. A self-toning photographic development emulsion comprising mainly silver chloride but no soluble silver salt as the light sensitive ingredient and a gold salt and a lead salt as self-toning ingredients.

70  
75  
80  
85  
90  
95

2. A self-toning photographic development emulsion comprising mainly silver chloride but no soluble silver salt as the light sensitive ingredient and a gold salt, a lead salt and a thiocyanate as self-toning ingredients.
3. A process for the production of self-toning photographic development emulsion comprising forming an emulsion containing essentially gelatine and silver chloride by precipitating the silver chloride from a soluble silver salt by means of a soluble chloride and then washing from the emulsion the non-silver salt formed by the reaction together with any excess soluble silver salts and soluble chloride, and then adding a solution containing gold salt and a lead salt as self-toning ingredients.
4. The process of claim 3 wherein a thiocyanate is also added as one of the self-toning ingredients.
5. A process for the production of a self-toning photographic development emulsion comprising forming an emulsion containing essentially

gelatine and silver chloride by precipitating the silver chloride in situ, washing from the emulsion any soluble salts, and adding to the emulsion as self-toning ingredients a gold solution made up by adding ammonium thiocyanate and a lead salt to gold chloride in the presence of gum arabic.

6. A method of producing a toned image which consists in exposing to light a paper bearing a self-toning photographic development emulsion comprising mainly silver chloride but no soluble silver salt as the light sensitive ingredient and a gold salt and a lead salt as self-toning ingredients, developing the exposed paper in a development solution to produce a reddish image and finally toning and fixing the image by immersing the print in a solution of sodium thiosulphate.

7. The method of claim 6 wherein an adurol development solution is employed.

8. The method of claim 6 wherein a hydro- 20 quinone development solution is employed.

WILLIAM AMBLER BERRY.